

## UNITED STATES PATENT OFFICE

2,269,601

PROCESS FOR THE MANUFACTURE OF  
ARTICLES RESISTANT TO GASEOUS COR-  
ROSIONRené Perrin, Paris, France, assignor to Société  
d'Electrochimie d'Electro-Metallurgie et des  
Acieries Électriques d'Ugine, Paris, France, a  
corporation of FranceNo Drawing. Application April 22, 1939, Serial  
No. 269,483. In France June 2, 1934

13 Claims. (Cl. 148—7)

This invention relates to a process for imparting to articles of alloyed metal the property of improved resistance to corrosion by a given gaseous substance especially at high temperatures. It is particularly adapted for rendering iron and steel articles resistant to corrosion by gaseous oxygen and sulphur compounds at high temperatures.

The present application is a continuation-in-part of my application, Serial No. 23,524, filed May 25, 1935.

It is known that certain alloying elements, such as aluminum, silicon, chromium and zirconium, when incorporated in suitable proportions in alloyed metals (especially in alloyed iron or steel) impart thereto a considerably increased resistance to chemical corrosion when exposed to gaseous substances such as oxygen or oxidizing mixtures (e. g. air, water vapor or carbon dioxide) or to gaseous sulphur compounds (e. g. sulphur dioxide or hydrogen sulphide) especially at high temperatures.

Protection against such gaseous corrosion is generally ascribed to the formation upon the surface of the alloyed metal, at the beginning of its utilization, of a film or coating of a metallic compound which is little or not at all attackable by the atmosphere in which the said metal is used; said film or coating serving to prevent said alloyed metal from being appreciably attacked subsequently by the corrosive constituents of said gaseous body. Metallic compounds having the properties required for this purpose are known to those skilled in the art. It is known, for instance, that a coating of alumina, formed upon the surface of an article of aluminum, will protect the latter from attack by the oxygen of the air, because, when adherent and of sufficient thickness, it prevents the base metal from coming into contact with the air. Such protective coating may be constituted principally of chromium oxide or aluminum oxide when the article to be protected is made of an alloy of chromium or aluminum and is to be subjected in use to an atmosphere containing oxygen at high temperature. It is understood that the protection afforded by such a film or coating is due not alone to the chemical nature thereof, but also to its properties of adherence, compactness and thickness. The term "base metal" is used herein to designate the chief component of the alloy (iron or steel for example) from the alloying metal (chromium or aluminum for example) which is used to protect such chief constituent from corrosion.

Heretofore a protective coating which fulfills the stated conditions has been obtained only by alloying with the base metal a very high proportion of alloying elements; which, besides involving excessive cost, has frequently the detrimental effect of imparting to the alloyed metal properties at variance with those it should possess. This occurs in the case of ferrous alloys when it is necessary to add thereto a large proportion (30% to 50%) of chromium or 10% or more of aluminum in order to render them corrosion-resistant to oxygen at high temperature, say of the order of 1000° C. Hence it is very difficult, and sometimes impossible, to regenerate such alloys (i. e. to subject them to a heat treatment for the purpose of restoring thereto properties which have deteriorated or disappeared in the course of mechanical operations, such as forging or the like) and consequently the range of application of such alloys is greatly restricted. Such chrome alloys, moreover, when maintained for a long time at high temperature, are liable to become fragile by reason of the growth of the grain of the ferrite.

It is obvious that, in the case of exposure to oxygen it is possible with an alloy of iron and a more readily oxidizable metal to form only the oxide of the more readily oxidizable metal by subjecting such alloy to a heating at high temperature at a partial pressure of oxygen of the order of that corresponding to the dissociation of the oxide of the more readily oxidizable metal at that temperature, since under these conditions the iron is practically not attacked. However, the use industrially of such extremely small partial pressures of oxygen involves difficulties so serious as to make it impracticable.

Moreover, the problem under consideration is not only to obtain at low cost a determined coating-composition, but also to produce a coating having the required properties of homogeneity, adhesiveness, compactness and thickness.

Contrary to previous practice and theory, the present invention makes possible the manufacture of corrosion resistant metallic articles of various shapes made of alloyed metals, especially ferrous alloys. This result is accomplished by adding to the base metal relatively small proportions of alloying elements and then treating the alloyed metal articles by a heating treatment under operating conditions that are thoroughly practical and economical, as hereinafter more fully described. The quantities of alloying elements required for accomplishing the above stated result by the process of this invention are

relatively much smaller than required for the production of corrosion resistant alloys by methods heretofore used. For example, by the treatment of this invention a steel containing only 12% chromium is rendered resistant to the oxidizing action of air when the article is heated to 1,000° C., whereas a chrome steel which has not been so treated must contain at least about 30% chromium, in order to make it equally resistant to oxidation under these same conditions. The amount of alloying element added to the ferrous base metal will vary according to the conditions under which the articles are to be used. Thus where chromium is the alloying metal and iron or steel the base metal and the article is intended to resist oxidation at 800° C. it was previously necessary to provide a chromium content of about 12%. By the treatment according to the invention a steel containing only 5.5% chromium is rendered resistant to the same extent to oxidation at 800° C.

This invention has for its essential object to produce upon an article made of an alloyed metal containing one or several alloying constituents a coating which will afford effective protection against corrosion by exposure to a determined gaseous body at high temperature. In case the alloy to be treated contains more than one alloying constituent, the said protective coating may comprise several compounds, corresponding respectively to the several alloying constituents. In any case but a single protective coating is, or need be, formed.

The present invention consists essentially in subjecting the article to be rendered corrosion resistant to the action, at a sufficiently high temperature, of an atmosphere containing the gaseous substance which the article is intended to resist in actual use or of an atmosphere containing a gaseous substance which when combined with the alloying metal gives rise to a coating capable of resisting to the gaseous atmosphere in which the article is to be actually used. If the article is to be used in an atmosphere containing oxygen, it is given a heating treatment in an atmosphere containing oxygen. The heating treatment is carried out at a temperature sufficiently high to cause a combination of the gaseous substance and the alloying element of the alloyed metal until a sufficiently thick compact coating is obtained. The temperature of the heating treatment is preferably at or above the temperature to which the article is to be subjected in use. However, the temperature of the heating treatment need not be as high as the intended temperature of use but need be only sufficiently high to cause a combination of the gaseous heating treatment substance and the alloying element. The heating treatment is conducted in an atmosphere containing the gaseous substance at a partial pressure above the dissociation pressure of the compound of the gaseous substance and the alloying element but low enough to avoid the formation of such an amount of the corresponding compound of the base metal as would unduly impair the effectiveness of the coating. The alloying element of the alloyed metal which combines with said gaseous substance is such that the compound formed thereby has a dissociation pressure below that of the compound formed by the action of said gaseous substance upon the base metal; the treatment being carried out in such manner that an ad-

herent compact and homogeneous coating of sufficient thickness is obtained.

Thus in order to obtain an article of chrome steel which is resistant to oxidation at high temperature (e. g. 1,000° C.), the process may be carried out advantageously by starting with a chrome steel having a chromium content insufficient in practice to be resistant to corrosion by itself at that temperature (say a 12% content of chromium) and subjecting this steel to a temperature near 1,000° C. at a pressure of oxygen between a fraction of a millimeter and several millimeters of mercury, say between  $\frac{1}{10}$  and 2 mm. of mercury for a sufficient time to produce a coating of chromium oxide thick enough to render the article corrosion resistant to oxygen at the temperatures and pressures under which it is intended to be used. The pressure of oxygen used during the heating treatment is kept insufficient to cause the formation of a coating rich in iron oxide, which coating would be permeable and would impair the effectiveness of the coating. If in the heating treatment just described the pressure of oxygen is  $\frac{1}{2}$  mm. of mercury, it will ordinarily be sufficient to carry out the heating treatment for a period of about 90 hours to produce a sufficiently thick compact homogeneous and adherent protective coating which will withstand satisfactorily the oxidizing action of air when the heat treated article is intended for resisting oxidation by air at 1,000° C. The heating treatment described will produce a coating which is adherent and not detachable from the article. By examination by X rays it is found that this coating is constituted by  $\text{Cr}_2\text{O}_3$  containing a small proportion of  $\text{Fe}_2\text{O}_3$ . The thickness of this coating is less than  $\frac{1}{16}$  mm.

The length of time required for forming a coating of proper thickness varies, of course, with varying conditions and depends also upon the particular use for which the article under treatment is destined. Therefore, in each case all details must be determined experimentally. This, however, is readily done. The maximum of oxygen pressure is likewise determined experimentally by a series of trials, in which the pressure is varied in a regular and progressive manner, as well understood by those skilled in the art.

In the treatment of an article of steel alloyed with say 4% of aluminum, the process may be carried out in a manner substantially similar to that described above. Obviously, in all cases the maximum pressure of oxygen at the determined temperature, to which the alloyed metal should be subjected during the heating treatment according to this invention, will depend upon the conditions attending the use for which the particular article is destined. Where, for example, chromium is the alloying metal, the protective coating may contain more oxide of iron (wherefore a higher partial pressure of oxygen at a determined temperature is permissible in the treatment according to this invention) when the article is intended for use at a lower temperature and with a lower pressure of oxygen. A protective coating may, for example, be formed at 1000° C. and with a partial oxygen pressure which is higher where the alloyed metal is to be used in air at 500° C. than when the same alloyed metal is to be used at 1000° C.

It should be observed that the protective coating will in fact contain not only the compound of the alloying metal (e. g. chromium oxide) but

also a small proportion of the corresponding compound of the base metal (e. g. iron oxide); in consequence whereof the corrosion resistance is, of course, correspondingly decreased. Therefore, the lower the temperature in which the article is to be used, the higher the permissible proportion of iron oxide.

The considerable importance of such a treatment as herein described is that it permits the utilization of articles made of alloys containing an alloying constituent in much smaller proportions than heretofore required, which alloys are, therefore, much less costly than those made heretofore for the same purpose, and which above all are more readily workable both in the hot and in the cold condition. Thus a steel with 12% of chromium is very easy to work and is easily heat treated to restore properties diminished by working while an iron alloy of 30% chromium is ferritic at all the range of temperatures, its properties cannot be restored by heat treatment and has moreover the disadvantage of becoming fragile by growth of the grain of ferrite during prolonged maintenance at a high temperature.

In order to improve the qualities of the protective coating and to accelerate its formation, the process according to the invention may be carried out by starting from a low pressure of treatment for the formation of the non-corrodible compound, for example of alumina and the pressure may be progressively increased after the first protective coating is formed. In this case one may even exceed without disadvantage, as soon as the protective coating is sufficiently thick, the pressure at which there is formed an appreciable proportion of the compound of the base metal, provided that this proportion is not so high as to unduly impair the effectiveness of the whole corrosion-resistant coating.

By increasing, during the treatment at a relatively high temperature according to this invention, the partial pressure of the gaseous substance, it is possible to cause the nature of the coating formed progressively to vary also. It is thus possible to use finally partial pressures of said gaseous substance which are relatively high and of the order of pressures to which the treated article is to be used under industrial conditions. Hence the final partial pressures to be employed in accordance with the invention are higher in the case of O and Fe, than the dissociation pressure of the oxide of the alloying element and that of FeO.

It is, therefore, possible to produce a coating of such a nature (due to its chemical composition and to its adherence, its homogeneity, its thickness, and its compactness) that the alloyed metal, when subjected to action of atmospheres common in industry, shows an extraordinarily increased corrosion-resistance. Moreover, the remarkable quality of resistance to corrosion above described is attained with alloyed metals containing alloying elements (such as Al or Cr) in proportions very much lower than those required hitherto in order to obtain equally high corrosion-resistance.

For example, to obtain a sufficiently thick coating of oxide on an iron or steel alloy containing Al, the alloyed metal is first subjected to a relatively low pressure of oxygen, which nevertheless is very high with respect to the dissociation pressure of oxides such as  $Al_2O_3$  (for example, 1.5-2 mm. of mercury); then, when the first coating is formed, the partial pressure of oxygen

may be increased slowly and progressively to 10 mm. of mercury. In this way, and without altering the resistance to corrosion of the coating, the thickness thereof may be increased in a relatively short time.

Inasmuch as the partial pressure of oxygen is very high relative to the dissociation pressure (at the temperature of the treatment) of the oxide of the alloying element added to the base metal, the formation of a compact coating of an oxide of sufficient thickness to be corrosion resistant to atmospheres now commonly used in industry may be effected in a comparatively short time. As has been already explained, the proper operating conditions (temperature, pressure, length of treatment, and the like) required for the production of a protective coating having the desired properties, are to be determined by suitable tests, regard being had in each case to the particular use for which the article under treatment is destined.

As a general rule, the following principles should be followed:

(1) The partial pressure of oxygen should be lower, the lower the proportion of alloying element added to the base metal.

(2) The treatment may be effected at higher partial pressure the lower the temperature of the treatment itself; thus temperature and pressure may be caused to vary inversely.

(3) The partial pressure of oxygen should be sufficiently high and the duration of the treatment should be sufficiently long so that a compact coating is obtained, which is thick enough to afford an efficacious protection against subsequent corrosion. It is not sufficient, in fact, to obtain a coating of a definite nature, it being also necessary that this coating be compact, adherent, and of sufficient thickness to insure corrosion-resistance. The partial pressure at which the treatment is carried out and the duration of the treatment will be, therefore, determined experimentally in each case.

When the coating is not sufficiently homogeneous (i. e. in a plane parallel to the outer surface of the coating), as explained below, the places at which a lack of such homogeneity exists will be manifested by the appearance of slits or cracks. When the coating is not sufficiently adherent, it has a tendency to separate from the base metal. When the coating is not sufficiently compact, there is liability of the formation of cracks under external influences and hence of corrosion. When the coating lacks the requisite thickness, there is a risk of its accidental removal.

It is to be understood in this connection that the "homogeneity" required for the purposes of this invention is not absolute or uniform homogeneity throughout the coating. What is required is that it should have a surface homogeneity; or, more precisely, the coating should be homogeneous in a plane which is parallel to the outer surface of the article. If, therefore, we consider two points of the coating, both being at the same depth from the external surface thereof, those points should show the same composition and structure.

Two examples of treatments with an indication of the results obtained will now be described.

In order to determine the oxidation resistance of an article of an iron aluminum alloy but not treated in accordance with the present invention, a cylindrical article of 50 mm. length and 8 mm.

diameter of iron aluminum alloy containing 4% aluminum was heated to 1000° C. for a period of eight hours in an atmosphere of pure dry oxygen under atmospheric pressure. It absorbed 270 cc. oxygen calculated at 0° C. and 760 mm. of mercury.

A like article of the same dimensions of the same alloy was first subjected to a heating treatment according to the present invention, which consisted in maintaining the article for 72 hours at 1000° C. in an atmosphere of oxygen at a partial pressure of 2 mm. mercury. The article was then tested in the same manner as was the first article—namely, by heating it to 1000° C. for a period of 8 hours in an atmosphere of pure dry oxygen under atmospheric pressure. Under these conditions of test, it absorbed only 5 cc. of oxygen, that is only  $\frac{1}{4}$  as much as the untreated article. Furthermore, the 5 cc. of oxygen absorbed also was less than that absorbed by another article identical in every way but made of steel containing 10% of aluminum but not treated according to the present invention, when tested under identical conditions.

An article of an iron chromium alloy containing 12% of chromium was tested for corrosion resistance with pure dry oxygen under atmospheric pressure at 1000° C. for a period of 8 hours. It absorbed 420 cc. of oxygen. A like article of the same dimensions of the same composition was given a heating treatment according to the present invention which consisted in maintaining the article for 72 hours at 1000° C. in an atmosphere of oxygen at a partial pressure of 2 mm. of mercury and was then tested by heating it to 1000° C. for a period of 8 hours in pure dry oxygen under atmospheric pressure. It absorbed only 10 cc. of oxygen in this test—that is to say only  $\frac{1}{42}$  as much as the untreated alloy. The 10 cc. of oxygen which was absorbed was less than that absorbed by a like article identical in every way but made of an alloy containing 30% of chromium when tested under the same conditions but untreated according to the present invention.

Amongst its industrial applications for the production of articles intended to resist high temperatures without being rapidly destroyed by the gases of the atmosphere to which they are exposed, may be mentioned for example furnace elements, pyrometers, wires for electrical resistances, a. s. o.

As previously pointed out, it is practically impossible, within reasonable limits of a specification, to set forth the exact conditions under which the heating treatment should be carried out to render an article corrosion resistant under every condition to which it may be subjected in actual use. One skilled in the art will have no difficulty in determining the optimum conditions of heating treatment for any particular intended use of the article. However, in order to set forth the invention as clearly as possible within reasonable limits of a specification, the following further explanation is given.

I have specifically referred to the use of chromium, aluminum, silicon and zirconium as alloying elements. The invention is not limited to these particular alloying elements but is applicable to other alloying elements which form corrosion resistant compounds when subjected to gaseous atmospheres, which corrosion resistant compounds have dissociation pressures lower than that of the corresponding compound of the base

metal and will form a sufficiently thick compact homogeneous and adherent protective coating on the article to protect it effectively from the attack of the gaseous atmosphere to which the article is to be subjected in use. Another alloying element which I may use in addition to aluminum, chromium, silicon, and zirconium previously mentioned is beryllium.

The amounts of alloying elements used will depend, among other factors, on the composition and temperature of the gaseous atmosphere in which the article is to be used. It also depends upon the amount of the particular alloying element which may be added to the particular base metal without unduly adversely affecting its physical properties and its ability to be worked into the desired shape. Considering chromium as the alloying element and iron or steel as the base metal for the production of articles intended to resist oxidation of air at atmospheric pressure and at temperatures of about 1000° C., the amount of chromium is preferably about 12%. The amount of chromium may be reduced, if the temperature of use is lowered or the partial pressure of the oxygen in the air is reduced or the degree of corrosion resistance required for the article is less than that ordinarily encountered. The resistance to corrosion of a ferrous alloy containing chromium in any appreciable amount, say as low as 3%, is increased by treatment according to the present invention. As a general statement, I shall use for most purposes not less than 12% of chromium in ferrous alloys intended for use in air under atmospheric pressure. The upper limit of chromium for ferrous alloys will probably not be above 30%, because to increase the chromium beyond this would be uneconomical or would adversely affect its fabricating properties too greatly. The range of chromium which will be used most generally in ferrous alloys is between about 12% and 17%.

With regard to aluminum as the alloying element, the preferred percentage for ferrous alloys is about 4%. I prefer to use not less than 1.5% in most cases and not over 6%. The silicon may be as low as 2% or as high as 7% but is preferably between 3% and 4%. The other alloying elements, if used, may be employed in percentages substantially less than are required to produce the desired protection where the article is not subjected to a previous heating treatment in accordance with the present invention. Thus, as a general statement, it may be said that  $\frac{1}{2}$  or  $\frac{1}{3}$  of the usual amount of alloying element is required according to the present invention.

The temperature of the heating treatment for producing the protective coating is preferably at or near the temperature of intended use of the article. This temperature, however, may be materially less than the temperature of intended use of the article, so long as the heat treating temperature is high enough to form the corrosion resistant compound of the alloying element. This temperature, as previously pointed out, will depend on the pressure of the gaseous substance in the heat treating atmosphere which causes corrosion. As a general statement, it may be said that if the chromium ferrous article is to be used for resisting oxidation of air at atmospheric pressure and at 1000° C., the temperature of the oxygen containing heating atmosphere will not be less than 600° C. nor higher than 1100° C.

The heating treatment temperature for aluminum containing ferrous alloy articles for use at temperatures of about 1000° C. in air at atmospheric pressure may be between 800° C. and 1200° C.

The time of the heating treatment for a ferrous alloy containing 4% of aluminum, in order to produce an article intended for use in air at atmospheric pressure and at a temperature of 1000° C. is generally between 10 and 100 hours where the partial pressure of oxygen in the heating atmosphere is 1 mm. of mercury. Generally the time of heating will be of the order of 80 hours. For a chromium containing ferrous alloy to be used under the same conditions, the time of heating treatment is generally also between 10 and 100 hours.

The partial pressure of oxygen in the heating atmosphere may be as low as  $\frac{1}{20}$  mm. of mercury or as high as 3 mm. of mercury, depending upon the heating treatment temperature, the proportion of alloying element and the intended use of the article.

It is to be emphasized again that the values which have been given are merely for illustrative purposes and it is not intended to limit the invention thereto.

The word "article" as used herein includes not only articles which have reached their final form but also articles which have not reached their final form.

The invention is not limited to the particular examples or to the preferred embodiments but may be otherwise embodied or practiced within the scope of the following claims.

I claim:

1. A process for improving the resistance of a metal to corrosion by a given gaseous substance, which comprises alloying with the said metal an alloying element which combines at high temperature with the gaseous substance to form a corrosion resistant compound having a dissociation pressure lower than that of the compounds of the base metal with said gaseous substance which are formed under the same heating conditions, and subjecting the alloyed metal to a heating pretreatment in an atmosphere containing the said gaseous substance at a partial pressure above the dissociation pressure of the said compound of the gaseous substance and the alloying element but below that at which the corresponding compound of the base metal forms in amount to materially impair the effectiveness of the coating wanted for the contemplated use of the alloy and below the partial pressure of said gaseous substance to which the alloyed metal is to be subjected in actual use, and at a temperature at which the alloying element combines with the gaseous substance to form the above said corrosion resistance compound, the heating being prolonged until a compact homogeneous and adherent protective coating of substantial thickness is obtained on the alloyed metal.

2. A process for improving the resistance of a metal to corrosion by a given gaseous substance, which comprises alloying with the said metal an alloying element which combines at high temperature with the gaseous substance to form a corrosion resistant compound having dissociation pressure lower than that of the compounds of the base metal with said gaseous substance which is formed under the same heating conditions, said alloying element being added in an amount insufficient to give by itself satisfactory resist-

ance to corrosion by the said gaseous substance under the intended conditions of use, and subjecting the alloyed metal to a heating pretreatment in an atmosphere containing said gaseous substance at a partial pressure above the dissociation pressure of the said compound of the gaseous substance and the alloying element but below that at which the corresponding compound of the base metal forms in amount to materially

5 impair the effectiveness of the coating and below the partial pressure of said gaseous substance to which the alloyed metal is to be subjected in actual use and at an elevated temperature at which the alloying element combines 10 with the gaseous substance to form the above said corrosion resistant compound, the heating being prolonged until a compact homogeneous and adherent protective coating of substantial thickness is obtained on the alloyed metal.

20 3. A process for improving the resistance of a metal to corrosion by a given gaseous substance, which comprises alloying with the said metal an alloying element which combines at high temperature with the gaseous substance to

25 form a corrosion resistant compound having dissociation pressure lower than that of the compounds of the base metal with said gaseous substance which are formed under the same heating conditions, and subjecting the alloyed metal

30 to a heating pretreatment in an atmosphere containing the said gaseous substance at a partial pressure above the dissociation pressure of the said compound of the gaseous substance and the alloying element but below that at which

35 the corresponding compound of the base metal forms in amount to materially impair the effectiveness of the coating and below the partial pressure of said gaseous substance to which the alloyed metal is to be subjected in actual use and at a temperature at which the alloying element combines with the gaseous substance to form the above said corrosion resistance compound, the heating being prolonged until a compact homogeneous and adherent protective coating of substantial thickness is obtained on the alloyed metal, and progressively increasing the partial pressure as the heat treatment is continued.

4. A process for improving the resistance of iron and steel to corrosion by oxidizing and sulphurous gases, which comprises alloying with a ferrous base metal an alloying element of the class consisting of chromium and aluminum, and subjecting the ferrous alloy to a heating pretreatment in an atmosphere containing the gas at a partial pressure above the dissociation pressure of any compound which forms by the reaction of the gas and the alloying element but below that at which the corresponding compound of the ferrous metal forms in amount to materially impair the effectiveness of the coating wanted for the contemplated use of the alloy and below the partial pressure of said gaseous substance to which the iron or steel is to be subjected in actual use and at a temperature at which the alloying element combines with the gas to form the above said corrosion resistant compound, the heating being prolonged until a compact, homogeneous and adherent protective coating of substantial thickness is obtained on the ferrous alloy.

5. A process for improving the resistance of iron and steel to corrosion by oxidizing and sulphurous gases, which comprises alloying with a ferrous base metal an alloying element of the

55

60

65

70

class consisting of chromium and aluminum in an amount insufficient to render the alloy resistant to corrosion by oxidizing and sulphurous gases under the intended conditions of use, and subjecting the ferrous alloy to a heating pretreatment in an atmosphere containing the gas at a partial pressure above the dissociation pressure of any corrosion resistant compound which forms by a reaction of the gas and the alloying element but below that at which the corresponding compound of the ferrous metal forms in amount to materially impair the effectiveness of the coating and below the partial pressure of said gaseous substance to which the iron or steel is to be subjected in actual use and at a temperature at which the alloying element combines with the gas to form the above said corrosion resistant compound, the heating being prolonged until a compact, homogeneous and adherent protective coating of substantial thickness is obtained on the ferrous alloy.

6. A process for improving the resistance of iron and steel to oxidation, which comprises alloying with the ferrous base, chromium in an amount insufficient to render the alloy resistant to oxidation under the intended conditions of use, and subjecting the ferrous alloy to a heating pretreatment in an atmosphere containing oxygen at a partial pressure above the dissociation pressure of chromium oxide but below that at which iron oxide forms in amount to materially impair the effectiveness of the coating and below the partial pressure of oxygen in the atmosphere to which the iron or steel is to be subjected in actual use and at a temperature at which chromium combines with oxygen, the heating being prolonged until a compact, homogeneous and adherent protective coating high in chromium oxide and low in iron oxide and of substantial thickness is obtained on the ferrous alloy.

7. A process for improving the resistance of iron and steel to oxidation, which comprises alloying with the ferrous base, aluminum in an amount insufficient to render the ferrous base resistant to oxidation under the intended conditions of use, and subjecting the ferrous alloy to a heating pretreatment in an atmosphere containing oxygen, at a partial pressure above the dissociation pressure of aluminum oxide but below that at which iron oxide forms in amount to materially impair the effectiveness of the coating and below the partial pressure of oxygen in the atmosphere to which the iron or steel is to be subjected in actual use and at a temperature at which aluminum combines with oxygen, the heating being prolonged until a compact, homogeneous and adherent protective coating high in aluminum oxide and low in iron oxide and of substantial thickness is obtained on the ferrous alloy.

8. A process for improving the resistance of iron and steel to oxidation, which comprises alloying with a ferrous base metal from 3% to 30% of chromium, and subjecting the ferrous alloy to a heating pretreatment in an atmosphere containing oxygen at a partial pressure above the dissociation pressure of chromium oxide but below that at which iron oxide forms in amount to materially impair the effectiveness of the coating and below the partial pressure of oxygen in the atmosphere to which the iron or steel is to be subjected in actual use, and at a temperature at which the chromium combines with oxy-

gen, the heating being prolonged until a compact homogeneous and adherent protective coating of chromium oxide of substantial thickness is obtained on the ferrous alloy.

5 9. A process for improving the resistance of iron and steel to oxidation, which comprises alloying with a ferrous base metal from 3% to 30% of chromium, and subjecting the so formed ferrous alloy to a heating pretreatment at a temperature between about 600 and 1100° C. in an atmosphere containing oxygen at a partial pressure above the dissociation pressure of chromium oxide but below that at which iron oxide forms in amount to materially impair the effectiveness of the coating and below the partial pressure of oxygen in the atmosphere to which the iron and steel is to be subjected in actual use, the heating being prolonged until a compact homogeneous and adherent protective coating of chromium oxide of substantial thickness is obtained on the ferrous alloy.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10405 10410 10415 10420 10425 10430 10435 104

temperatures of the order of about 1000° C., which comprises subjecting the steel to a heating pre-treatment at about 800 to 1200° C. in an atmosphere containing oxygen at a partial pressure of about .02 to 3 millimeters of mercury and above the dissociation pressure of aluminum oxide but below that at which iron oxide forms in an amount materially to impair the effectiveness of

the protective coating which is formed and continuing such heat treatment until a compact homogeneous and adherent protective coating high in aluminum oxide and low in iron oxide and of substantial thickness is formed on the surface of the steel.

RENÉ PERRIN.